

# United States Patent

Watts

[15] 3,705,615

[45] Dec. 12, 1972

[54] METAL CASTING PROCESSES WITH  
VACUUM AND PRESSURE

[72] Inventor: Claude H. Watts, Mayfield Heights,  
Ohio

[73] Assignee: Precision Metalsmiths, Inc.

[22] Filed: Dec. 9, 1970

[21] Appl. No.: 96,517

[52] U.S. Cl. .... 164/62, 164/65, 164/255,  
164/256

[51] Int. Cl. .... B22d 27/14, B22d 27/15

[58] Field of Search.... 164/62, 65, 61, 255, 256, 258

[56] References Cited

## UNITED STATES PATENTS

1,070,500 8/1913 Mackenzie ..... 164/258

|           |         |                      |          |
|-----------|---------|----------------------|----------|
| 2,133,634 | 10/1938 | Rohn.....            | 164/258  |
| 3,336,970 | 8/1967  | Watts et al. ....    | 164/62   |
| 3,620,296 | 11/1971 | Barbieri et al. .... | 164/62 X |

Primary Examiner—Robert D. Baldwin

Attorney—Watts, Hoffmann, Fisher & Heinke

[57] ABSTRACT

A gas permeable mold, preferably an investment mold, is cast under a vacuum. The pressure on the molten metal exposed through the opening of the mold is raised to atmospheric pressure after casting, and a vacuum is applied to the outside of the mold during solidification of the metal.

12 Claims, 1 Drawing Figure



PATENTED DEC 12 1972

3,705,615



INVENTOR.  
CLAUDE H. WATTS

BY *Watts, Hoffmann,  
Fisher & Heimke*  
ATTORNEYS.

## METAL CASTING PROCESSES WITH VACUUM AND PRESSURE

### BACKGROUND OF THE INVENTION

The present invention relates generally to metal casting processes, and more specifically to methods of casting investment molds, including both shell molds and bulk investment molds.

The invention is particularly concerned with providing methods for producing sound investment castings made of aluminum alloys and other metals which are subject to similar defects. Investment cast aluminum alloys are recognized to be especially susceptible to air entrapment and porosity, and in the past these conditions have been a major cause of rejected castings. In some instances, for example, when casting Type 355 and Type 356 aluminum alloys, a very high rejection rate of from 75 percent to 90 percent has been experienced. Another problem encountered in the investment casting of metals such as aluminum alloys is that of the metal retracting from the surfaces of the investment mold during solidification. This condition is frequently referred to as "draw-back."

### SUMMARY OF THE INVENTION

According to the present invention, there is provided a method of casting a gas permeable mold, such as an investment mold, comprising the steps of introducing molten metal while under a vacuum into an opening of the mold to fill a cavity, thereafter increasing the pressure on the molten metal through the mold opening, and applying a vacuum to the outside of the mold during solidification of the metal.

According to a more preferred aspect of the present invention, there is provided a method of casting a gas permeable mold, such as an investment mold, which comprises the steps of placing the mold in a mold chamber so that the opening of the mold communicates with a vacuum casting chamber which is sealed from the mold chamber, evacuating the vacuum casting chamber and then introducing molten metal into the opening of the mold to fill a cavity, thereafter restoring the casting chamber to atmospheric pressure while the metal in the mold is still molten, and applying a vacuum to the outside of the mold by evacuating the mold chamber prior to solidification of the metal, and more preferably prior to introducing the metal into the mold.

The new methods provided by the invention can be used to cast many different kinds of metals, and may be found particularly advantageous in producing castings having thin wall sections. The new methods are especially suited for casting aluminum alloys and the like which are subject to air entrapment, porosity and draw-back.

Other advantages and a fuller understanding of the invention will be had from the following detailed description and the accompanying drawing.

### BRIEF DESCRIPTION OF THE DRAWING

The drawing is a diagrammatical, vertical cross-sectional view showing an apparatus for carrying out the method of this invention.

### DESCRIPTION OF THE PREFERRED EMBODIMENT

The illustrated apparatus is the invention of Timothy L. Coghill and was developed after the date of the present invention. The apparatus is disclosed as the best known mode of practicing the invention, but no claim of inventorship is made thereto.

The illustrated apparatus comprises an enclosure 10 which is adapted to define a mold chamber 11 and a vacuum casting chamber 12. The mold chamber 11 is connected through a conduit 13 and a valve (not shown) to a suitable vacuum source, such as a vacuum pump or line. The vacuum casting chamber 12 also is connected to a suitable vacuum source through a conduit 14 and a valve (not shown). The valves in the conduits 13, 14 are three-way valves which can be actuated to connect the chambers 11, 12 to vacuum source and to the atmosphere.

A platform 20 is provided within the chamber 11 for supporting a mold. The platform 20 may be comprised of a metal plate 21 on which is disposed a gasket 22. Suitable gaskets may be made from asbestos pads, insulation or blankets formed of refractory fibers, such as aluminasilica fibers, and the like. A hole 23 is formed through the plate 21 and the gasket 22, and the plate 21 is supported above the bottom of the chamber 11 by suitable supports 24. The height of the supports 24 is preferably adjustable so that the top of the mold supported on the platform can be positioned in the desired plane.

As shown, the enclosure 10 includes a lower section 30 which defines the mold chamber 11 and an upper section 31 which defines the vacuum casting chamber 12. A suitable sealing gasket 32 is provided between the two sections of the enclosure. The upper section 31 can be separated from the lower section 30 to permit a mold to be placed into and removed from the mold chamber 11. The upper section 31 includes a window 33 through which an operator can observe the casting operation.

A ladle 35 is pivotally mounted in the casting chamber 12 for use in pouring metal into a mold supported on the platform 20 in the mold chamber 11. A handle (not shown) which is used to tip the ladle extends through a side of the enclosure section 31. The upper section 31 of the enclosure 10 is provided with a plate 36 which can be removed to fill the ladle 35.

An illustrative investment mold which can be cast by the practice of this invention is generally designated by reference numeral 45. The mold 45 is comprised of a refractory body 46 having an opening 47, a central passage 48, and a plurality of pattern cavities 49 which are gated into the passage 48. As shown, a core 50 is positioned within the mold passage 48. The core 50, which may be formed of refractory material, has a closed end and an open end. A peripheral rim or step 51 is formed at the lower, open end of the core. The rim or step 51 serves to center the core 50 within the mold body 46 and substantially fills the passage 48 so that little or no molten metal can squeeze past the core when the mold is cast. A refractory pouring basin or collar 52 is shown positioned on the top of the mold 45 around its opening 47.

The refractory mold body 46 may be made by conventional investment molding techniques. A plurality

of patterns which are replicas of the parts to be cast in metal, including the necessary gates and risers, and which are formed of an expendable material, such as wax, are attached to a central sprue member to form what is known as a "set-up" or "tree." The set-up or tree is placed within a heat-resistant flask 53 which is preferably perforated and the flask is filled with a cementitious refractory material known as the "investment" which hardens at room temperature around the set-up or tree. The investment material may be a gypsum bonded refractory material which consists essentially of cristobalite and fine silica powder together with accelerators and retarders to adjust the setting time. After hardening, the set-up is removed from the mold body 46 to form the central passage 48 and the mold cavities 49.

In carrying out the practice of this invention, the mold 45 is placed in the chamber 11 on the platform gasket 22 and the core 50 is positioned with its open end over the hole 23 of the platform. The mold chamber 11 is then sealed from the vacuum casting chamber 12 with the opening 47 of the mold in communication with the vacuum casting chamber. This is accomplished by a metal ring 60 which surrounds the upper end of the mold and is supported by a shoulder 61 of the lower enclosure portion 30. A rubber sealing ring 62 or the like is disposed between the ring 60 and the shoulder 61. The seal is completed by a ring 63 which rests on the upper end of the mold 45 and on the ring 60. The ring 63 may be made of asbestos, rubber or other similar material.

When the mold 45 has been positioned in the manner described, the ladle 35 is filled with molten metal and a vacuum is drawn in the casting chamber 12 to evacuate the interior of the mold. In accordance with conventional practice, the metal is usually degassed prior to being placed in the ladle, and therefore the metal can be introduced into the mold 45 as soon as the desired vacuum has been obtained in the chamber 12. The degree of vacuum in the chamber 12 can be varied depending upon such factors as the kind of metal being cast, the amount of metal, the size of the mold, etc. A typical vacuum used for casting aluminum alloys is from 26 to 28 inches of mercury below atmospheric pressure.

After the molten metal has been poured into the mold 45, the pressure in the casting chamber 12 is raised, preferably by relieving the vacuum and opening the chamber to atmospheric pressure. Atmospheric pressure on the molten metal exposed in the mold opening 47 acts to force the molten metal into the mold cavities to promote a complete fill and aids in preventing draw-back as the metal subsequently solidifies.

A vacuum is drawn in the mold chamber 11 prior to solidification of the metal and preferably at the same time that the vacuum is drawn in the casting chamber 12. The metal in the mold opening is maintained at atmospheric pressure and the vacuum applied to the outside of the mold is continued during at least partial solidification of the metal. The degree of vacuum in the chamber 11 which has been found sufficient successfully to cast metals such as aluminum alloys is usually 15 inches or more of mercury below atmospheric pressure. It is believed that the effectiveness of the vacuum around the mold may be the result of removing air from

the pores of the mold and thereby preventing any such air from coming out of the pores prior to and during solidification. Whatever the explanation, it has been found that the application of the vacuum to the outside of the mold while the metal is under pressure through the mold opening results in the production of sound castings which are free of the defects heretofore encountered.

The solidification characteristics of the metal are affected by the rate of cooling and the temperature of the molds at the time of introducing the metal. In order to promote a complete fill of the mold cavities, it may be desired to cast the molds while they are hot. For example, when casting Types 355 and 356 aluminum alloys, investment molds are frequently at a temperature in the range of from about 300° to 800°F., and preferably at a temperature of approximately 400°F. In other instances, for example, when producing castings having thick or heavy wall sections, it may be desirable to pour the molds at room temperature in order to chill the heavy wall sections as rapidly as possible.

An example of the invention involved the casting of an investment mold substantially as shown in the drawing, the mold having been made by the conventional practice described above. A dome-shaped core was spaced approximately one-half inch from the inside surface of the mold. The mold was cast at a temperature of 400°F. with Type 356 aluminum alloy which was poured at a temperature of 1,300°F. The nominal composition of the alloy was 0.3 percent magnesium, 7 percent silicon and the balance aluminum. A vacuum of 26 inches of mercury below atmospheric pressure was drawn in the casting chamber prior to introducing the metal into the mold. Immediately after casting the mold, the casting chamber was restored to atmospheric pressure and a vacuum of from 15 to 20 inches of mercury below atmospheric pressure was maintained in the mold chamber 11. The metal was allowed to solidify for 2 to 3 minutes before releasing the vacuum in the mold chamber. The castings which were produced were found to be free of air entrapment and draw-back. Similar molds were cast with Type 356 aluminum alloy following the same procedure except for the elimination of the step of applying a vacuum to the mold body during solidification. The castings which were produced were unsatisfactory because of extreme porosity and severe drawback.

As used herein, the term "investment molds" is meant to include bulk or solid molds of the type shown in the drawing and ceramic shell molds. It is to be understood that the methods provided by this invention are not limited to the casting of investment molds of any specific type or which are made of a particular refractory material, and that the mold 45 has been disclosed only for the purpose of setting forth one specific example of the new casting technique. The methods which have been described may be used to advantage in casting bulk or solid type investment molds which are not provided with cores such as shown at 50, ceramic shell molds, and other types of gas permeable molds, including sand molds, etc.

Many modifications and variations of the invention will be apparent to those skilled in the art in the light of the foregoing disclosure. Therefore, it should be understood that, within the scope of the appended claims,

the invention can be practiced otherwise than as specifically shown and described.

What is claimed is:

1. In the casting of a gas permeable mold having an opening into which molten metal is poured to fill a cavity of the mold, a method comprising the steps of:

- a. evacuating the cavity of the mold and introducing molten metal while under a vacuum into the mold opening to fill the cavity,
- b. thereafter increasing the pressure on the molten metal through the mold opening, and
- c. Applying a vacuum to the outside of the mold prior to solidification of the metal.

2. In the casting of a gas permeable mold having an opening into which molten metal is introduced to fill a cavity of the mold, a method comprising the steps of:

- a. applying a vacuum to the opening of the mold,
- b. introducing molten metal under a vacuum into the mold opening to fill the cavity,
- c. thereafter relieving the vacuum applied to the mold opening so that the pressure on the molten metal in the mold is increased, and,
- d. applying a vacuum to the outside of the mold prior to solidification of the metal.

3. In the casting of a gas permeable mold having an opening into which molten metal is introduced to fill a cavity of the mold, a method comprising the steps of:

- a. removing air from the inside of the mold through the mold opening,
- b. introducing molten metal under a vacuum into the mold opening to fill the cavity,
- c. thereafter exposing the opening of the mold to atmospheric pressure while the metal is still molten,
- d. applying a vacuum to the outside of the mold prior to solidification of the metal, and
- e. maintaining the mold opening exposed to atmospheric pressure and continuing to apply a vacuum to the outside of the mold as the metal at least partially solidifies.

4. A method as claimed in claim 3 wherein the vacuum is applied to the outside of the mold prior to the step of introducing molten metal into the mold opening.

5. In the casting of a gas permeable mold having an opening into which molten metal is introduced to fill a cavity in the mold, a method comprising the steps of:

- a. mounting the mold so that its opening is in communication with a vacuum casting chamber,
- b. evacuating the chamber and then introducing molten metal into the mold opening to fill the cavity,
- c. increasing the pressure in the chamber while the metal in the mold is still molten,
- d. applying a vacuum to the outside of the mold prior to solidification of the metal, and
- e. continuing the application of the vacuum as the metal at least partially solidifies.

6. A method as claimed in claim 5 wherein the vacuum is applied to the outside of the mold before introducing the molten metal into the mold opening.

7. In the casting of a gas permeable mold having an opening into which molten metal is introduced to fill a cavity of the mold, a method comprising the steps of:

- a. mounting the mold in a mold chamber with the opening of the mold communicating with a vacuum casting chamber which is sealed from the mold chamber,
- b. evacuating the vacuum casting chamber and then introducing molten metal into the mold opening to fill the cavity,
- c. thereafter restoring pressure to the vacuum casting chamber while the metal in the mold is still molten, and
- d. evacuating the mold chamber prior to solidification of the metal.

8. A method as claimed in claim 7 wherein the mold chamber is evacuated before the step of introducing the metal into the mold opening.

9. A method as claimed in claim 7 including the step of preheating the mold before placing it in the mold chamber.

10. In casting a gas permeable mold having an opening into which molten metal is introduced to fill a cavity of the mold, a method comprising the steps of:

- a. evacuating the cavity of the mold and introducing molten metal under vacuum into the mold opening to fill the cavity,
- b. thereafter causing the pressure on the molten metal which is exposed through the opening of the mold to be increased,
- c. providing a sealed chamber around the mold,
- d. evacuating the chamber to apply a vacuum to the outside of the mold before the metal in the mold cavity has solidified, and
- e. continuing to apply the vacuum to the outside of the mold and to maintain the increased pressure on the metal through the mold opening while the metal at least partially solidifies.

11. A method as claimed in claim 10 including the step of heating the mold so that it is hot during introduction of the molten metal.

12. In the casting of a gas permeable mold having an opening into which molten metal is introduced to fill a cavity of the mold, a method comprising the steps of:

- a. mounting the mold so that its opening is in communication with a vacuum casting chamber,
- b. evacuating the casting chamber and then introducing molten metal into the mold opening to fill the cavity,
- c. thereafter increasing the pressure on the metal in the mold through the mold opening,
- d. providing a sealed chamber around the mold,
- e. evacuating the sealed chamber to apply a vacuum on the outside of the mold before the metal in the mold cavity has solidified, and
- f. continuing to apply the vacuum to the outside of the mold and to maintain the increased pressure on the metal through the mold opening while the metal at least partially solidifies.

\* \* \* \* \*